

1,007,146.

E. J. SCHRODER.  
PREPARED ROOFING.  
APPLICATION FILED SEPT. 9, 1910.

Patented Oct. 31, 1911.

Fig. 1.



Fig. 2.



Witnesses

Robert H. Weir

George L. Chindahl

Inventor:

Edward J. Schroder  
By Luther L. Miller, Atty.

# UNITED STATES PATENT OFFICE.

EDWARD J. SCHRODER, OF CHICAGO, ILLINOIS.

## PREPARED ROOFING.

1,007,146.

Specification of Letters Patent. Patented Oct. 31, 1911.

Application filed September 9, 1910. Serial No. 581,261.

To all whom it may concern:

Be it known that I, EDWARD J. SCHRODER, a citizen of the United States, residing at Chicago, in the county of Cook and State 5 of Illinois, have invented certain new and useful Improvements in Prepared Roofing, of which the following is a specification.

One of the objects of this invention is to provide a prepared or composition roofing 10 having an outer protective layer adapted effectively to resist the action of moisture, heat and corrosive gases and vapors.

A further object of the invention is to impart to prepared roofing a permanent, attractive color.

These objects I attain by placing upon a roofing body of any suitable or preferred character a layer of crushed slate, the slate being rolled upon the roofing body so as 20 firmly to attach the slate particles to said body, and to give to the slate coating a substantially smooth exterior surface. Slate being of laminated structure, the particles of crushed slate partake of the general character 25 of flakes, matching together so as completely to cover the asphalt or other waterproofing material located below, thereby effectively protecting said asphalt from rain and snow and from the corrosive fumes and 30 gases to which roofing is subjected when used upon fertilizer and chemical manufacturers, etc. Moreover, by the use of the slate covering a permanent and uniform color is obtained without added expense.

35 In the accompanying drawings, Figure 1 is a fragmental top plan view of prepared roofing embodying the features of my invention. Fig. 2 is a cross-sectional view, more or less diagrammatic, of said roofing.

40 Roofing embodying my invention may comprise a body of any suitable or preferred character; that herein shown by way of example consists of a sheet 1 of felt saturated with a suitable waterproofing material, as, 45 for instance, asphalt; a layer 2 of asphalt placed upon the felt; a sheet 3 of burlap saturated with waterproofing material and superposed upon the layer 2; and a coating 50 4 of asphalt or the like placed upon the burlap. At a suitable point in the manufacture of the roofing I place upon the roofing body a layer of crushed slate and press the slate particles into close contact with

the asphalt coating 4 by means of suitable rolls. The slate covering is represented diagrammatically at 5 in the drawings. Slate being of stratified or laminated texture, as distinguished from the crystalline form, the particles of crushed slate consist of flakes or laminae, which when rolled lie 60 substantially parallel with the plane of the roofing body, and thus impart to the finished product an approximately smooth outer surface. When the slate is rolled, some of the asphalt is forced into the interstices between the slate flakes, and to the asphalt thus exuded other flakes become attached, the asphalt coating 4 thus becoming completely covered with slate.

As indicated in the drawings, some of the flakes of slate match together, these being held in place by the asphalt below; and some of the flakes overlap the crevices existing between the other slate fragments, such overlapping pieces being retained in place 75 by the asphalt forced into said crevices during the rolling process. Because of its continuous character, the slate coating gives a uniform color to the roofing.

In roofing as heretofore constructed, the 80 gravel, sand or crystalline material does not effectively protect the asphalt or other adhesive layer below it, and consequently the asphalt exposed to the action of the weather and corrosive acids deteriorates and loses 85 its power of holding in place the gravel or other material composing the outer layer of the roofing. When the gravel thus released is washed or blown away, other portions of the asphalt become exposed, and 90 the process of deterioration goes on at an increasing rate. In roofing embodying my invention, however, the slate covering efficiently protects the asphalt from moisture and injurious fumes, and therefore is itself 95 effectively retained in place by the asphalt.

The slate imparts to the finished article the natural color of the slate, which color is permanent and uniform and is, of course, obtained without additional expense.

100 It will be understood that my invention is applicable to composition roofing in roll, sheet or shingle form.

I claim as my invention:

105 Prepared roofing consisting of a body having a coating of adhesive waterproofing

material, and an outer protective coating of crushed slate, the flakes of slate being rolled into contact with the adhesive material, said flakes lying substantially parallel with the adhesive coating, said flakes being matched together and overlapped so as to cover the adhesive material; the layer of slate par-

ticles providing an approximately smooth outer surface for the roofing.

EDWARD J. SCHRODER.

Witnesses:

FRANK C. STRASSER,  
EBEN R. CHRISTENSEN.